

[54] **RESISTIVE SUBSTRATE FOR THERMAL PRINTING RIBBONS COMPRISING A MIXTURE OF THERMOSETTING POLYIMIDE, THERMOPLASTIC POLYIMIDE, AND CONDUCTIVE PARTICULATE MATERIAL**

[75] Inventor: Arthur E. Graham, Lexington, Ky.

[73] Assignee: International Business Machines Corporation, Armonk, N.Y.

[21] Appl. No.: 333,348

[22] Filed: Dec. 22, 1981

[51] Int. Cl.<sup>3</sup> ..... B41J 31/00

[52] U.S. Cl. ..... 400/120; 400/198; 400/241.1; 428/914

[58] **Field of Search** ..... 400/118, 119, 120, 198, 400/241.1, 241.2; 428/448, 473.5, 914; 427/148

[56] **References Cited**

**U.S. PATENT DOCUMENTS**

|           |         |                  |                   |
|-----------|---------|------------------|-------------------|
| 2,713,822 | 7/1955  | Newman           | ..... 101/460 X   |
| 3,377,598 | 4/1968  | Borman           | ..... 400/198 X   |
| 3,551,200 | 12/1970 | Stivers          | ..... 428/473.5 X |
| 3,744,611 | 7/1973  | Montanari et al. | ..... 400/120     |
| 3,868,351 | 2/1975  | Hand et al.      | ..... 428/473.5 X |
| 4,103,066 | 7/1978  | Brooks et al.    | ..... 400/120 X   |

|           |         |                 |                   |
|-----------|---------|-----------------|-------------------|
| 4,236,834 | 12/1980 | Hafer et al.    | ..... 400/120     |
| 4,253,775 | 3/1981  | Crooks et al.   | ..... 400/119     |
| 4,269,892 | 5/1981  | Shattuck et al. | ..... 400/241.1 X |
| 4,309,117 | 1/1982  | Chang et al.    | ..... 400/241.1   |
| 4,345,845 | 8/1982  | Bohnhoff et al. | ..... 400/120     |

**FOREIGN PATENT DOCUMENTS**

1221489 2/1971 United Kingdom ..... 400/241.2

**OTHER PUBLICATIONS**

*IBM Technical Disclosure Bulletin*, "Thermal Efficiency Improvement by Anodization", Bowlds et al., vol. 24, No. 3, Aug. 1981, pp. 1356-1357.

*Primary Examiner*—Ernest T. Wright, Jr.  
*Attorney, Agent, or Firm*—John A. Brady

[57] **ABSTRACT**

Disclosed is a thermal transfer medium which comprises a mixture of a thermosetting polyimide, a thermoplastic polyimide, and graphite. It has a steel support layer and an intermediate layer of silicon dioxide. An outer layer on the steel is the thermal ink. The mixture is applied as a dispersion with a precursor of the thermosetting polyimide. The ribbon may be recoated at the typing station by applying a hot melt of the ink.

**12 Claims, 1 Drawing Figure**



U.S. Patent

Dec. 20, 1983

4,421,429



**RESISTIVE SUBSTRATE FOR THERMAL  
PRINTING RIBBONS COMPRISING A MIXTURE  
OF THERMOSETTING POLYIMIDE,  
THERMOPLASTIC POLYIMIDE, AND  
CONDUCTIVE PARTICULATE MATERIAL**

**DESCRIPTION**

**CROSS REFERENCE TO RELATED  
APPLICATION**

Application Ser. No. 333,349, filed Dec. 22, 1981 the same date as this application, entitled "Silicon Dioxide Intermediate Layer In Thermal Transfer Medium," by Patsy M. Bowlds, Bruce M. Cassidy, Arthur E. Graham, Robert J. Haljak, Deh C. Tao, and Donald W. Stafford and assigned to the same assignee to which this application is assigned, is directed to a silicon dioxide intermediate layer. The preferred embodiment of this invention includes the silicon dioxide intermediate layer.

**TECHNICAL FIELD**

This invention is to ribbons for non-impact, thermal printing by resistive heating in the ribbon. Ink is transferred from the ribbon to paper at localized areas at which heat is generated. Localized heating may be obtained, for example, by contacting the ribbon with point electrodes and a broad area contact electrode. The high current densities in the neighborhood of the point electrodes during an applied voltage pulse produce intense local heating which causes transfer of ink from the ribbon to a paper or other substrate in contact with the ribbon.

**BACKGROUND ART**

Printing by thermal techniques of the kind here of interest is known in the prior art, as shown, for example, in U.S. Pat. Nos. 2,713,822 to Newman, 3,744,611 to Montanari et al, and 4,269,892 to Shattuck et al.

Various materials are employed as the major structural material of the resistive layer. Thus, for example, U.S. Pat. No. 4,103,066 to Brooks, et al is directed to polycarbonate resins and U.S. Pat. No. 4,269,892 to Shattuck, et al is directed to polyester resins and polyester and urethane resins. Both disclose conductive carbon black dispersed in the resin to provide a degree of electrical resistivity desired.

In certain thermal printing systems, resistance of the ribbon to permanent change from the heat of printing is sought. Particularly where the ribbon is to be reused, heat-resistance is critical since the ribbon must both retain its physical characteristics and not be significantly deformed as by stretching. Polyimide is known to be resistive to heat, and U.S. Pat. Nos. 4,236,834 to Hafer, et al and 4,253,775 to Crooks, et al teach reusable systems employing polyimide.

The teachings of both of these patents are prior art to the invention of this application. Both are directed to reusable elements for thermal printing for which this invention is also well suited. The Hafer, et al patent discloses a resistive layer of polyimide and carbon laminated to a thin aluminum layer. The Crooks, et al patent discloses a resistive layer "comprised of conductive particles, for example, of graphite, suspended in a high temperature polymer, for example, Kapton." Kapton is a brand name for a stable polyimide.

This invention also employs polyimide as the resin material of the conductive layer of a thermal transfer

medium. In accordance with this invention, however, a blend of thermosetting and thermoplastic polyimides are employed to achieve, in addition to temperature stability, excellent electrical resistivity, as well as good strength and, where filled with graphite, excellent abrasion resistance.

**DISCLOSURE OF INVENTION**

In accordance with this invention the resistive layer 10 of a thermal transfer medium is a mixture of a thermosetting polyimide and a thermoplastic polyimide with a particulate conductive material, which in the preferred embodiment is graphite. Also in the preferred embodiment the resistive layer of blended polyimides is laminated to a very thin layer of silicone dioxide which provides heating properties near the printing area which are extremely important in an actual printing system.

The thermosetting polyimide is commercially available 20 as a liquid in a high-boiling organic solvent system. Advantageous properties of this polyimide are the following: (1) Excellent adhesion to metal and pigments compared to the thermoplastic polyimide; (2) Good abrasion resistance compared to the thermoplastic polyimide; and (3) Available as a liquid. Disadvantageous properties of the thermosetting polyimide are the following: (1) Solubility is by high-boiling solvents; (2) Poor electric insulator compared to the thermoplastic polyimide; and (3) Poor vehicle for pigment dispersions 30 because the pigments float.

The thermoplastic polyimide is commercially available 35 as a solid, and is known to be readily soluble in tetrahydrofuran (THF) and many other organic solvents. Advantageous properties of this polyimide are the following: (1) Allows wide choice of processing solvents; (2) Good electric resistance compared to the thermosetting polyimide; (3) Excellent binder for pigment dispersion, yielding no pigment streaking, non-uniformity and the like; and (4) Readily imbibes solvent 40 to take on a stretchable consistency. Disadvantageous properties of the thermoplastic polyimide are the following: (1) Poor adhesion to metal and pigments compared to the thermosetting polyimide; and (2) Poor abrasion resistance compared to the thermosetting polyimide.

A blend of the two with appropriate solvents and a 45 filler of particulate conductive material such as graphite is solid to the touch within 60 seconds at room temperature. After subsequent treatment at elevated temperature to set the thermosetting resin, a thermal ribbon is achieved having the necessary physical integrity and 50 exceptionally good resistance to degradation during use in the thermal printing process. The element is strong and abrasion resistant, and has electrical resistivity well suited to the thermal printing.

**BRIEF DESCRIPTION OF THE DRAWING**

A preferred embodiment of this invention is described 55 in detail with reference to the accompanying drawing, which shows a side view of the reinkable ribbon.

**BEST MODE FOR CARRYING OUT THE  
INVENTION**

The preferred and best embodiment of this invention is a four-layer laminated ribbon 1 of regular cross-section particularly suited to be reinked and reused. The

bottom, resistive layer 3 is a blend of polyimides with conductive, particulate graphite, which acts as a resistive layer. Resistive layer 3 is 0.3 mil in thickness (0.3 thousandth of an inch; 0.000762 centimeters). The next layer 5 is an 80 angstroms thick layer of silicon dioxide. The layer 7 next to the silicon dioxide is a stainless steel conductive and support layer 7. The conductive and support layer 7 is 0.5 mil in thickness (0.001270 centimeters). Finally, on the steel layer 7 is an ink layer 9 flowable in response to heat created by electric current applied from the outside of the resistive layer 3.

The essential contribution of this invention is in the blend of polyimide resins employed in the resistive layer 3. Printing is effected by known techniques in which the resistive layer 3 is contacted with point electrodes, such as electrodes 16 in U.S. Pat. No. 4,345,845 to Bohnhoff et al, which is illustrative of pertinent, known printing techniques. The resistive layer 3 or the steel layer 7 is contacted with a broad area electrode, such as collector contact 28 in the foregoing patent to Bohnhoff et al. The point electrodes (16 in the foregoing patent to Bohnhoff et al) are selectively driven in the form of the images desired with sufficient current to produce local heating which causes transfer of ink from ribbon 1 to a paper or other substrate (14 in the foregoing patent to Bohnhoff et al) in contact with the ribbon 1.

The stainless steel layer 7 provides physical strength, which is particularly important in the preferred embodiment since the ribbon 1 is intended to be used again and again. The steel layer 7 also is highly conductive and therefore provides a path of low electrical resistance from the area of the point contact electrodes to the broad area electrode. Accordingly, the area of primary electrical heat from current flow will be near the point electrodes. The use of steel or other metal as a thermal ribbon lamination and for these purposes forms no part of the contribution of this invention. The preferred embodiment steel is alloy 304, a chromium-nickel austenitic stainless steel.

The silicon dioxide layer 5, situated between the resistive layer 3 and the steel layer 7, is the essential contribution of the invention to which the application entitled "Silicon Dioxide Intermediate Layer In Thermal Transfer Medium," described in the first paragraph of this application, is directed. Silicon dioxide generally is an electric insulator. The very thin layer 5 of silicon dioxide does conduct, but in a manner of a high resistance. Accordingly, much of the heat generated in the ribbon during printing appears to be generated at the silicon dioxide layer 5 opposite each point electrode delivering current. This area is directly in contact with the steel layer 7, a good thermal conductor to the ink layer 9.

The ink layers 9 may be conventional. Two alternative embodiments will be described.

#### PROCESS OF MANUFACTURE

##### Resistive Layer Formula

The thermosetting polyimide: This material in the three formulas to be described is an ingredient of DuPont PI 2560, a trademark product of E. I. DuPont de Nemours Co. This is sold commercially as a solution described as  $37 \pm 1.5\%$  by weight solid precursor of polyimide, dissolved in about 47% by weight N-methyl-2-pyrrolidone (NM2P) and 16% by weight xylene. It has a density of 1.43 grams per cubic centimeter, and the material polymerizes further after loss of the solvents at temperatures of 335° F. The final product is firm and

massive, and does not soften appreciably at high temperatures.

The thermoplastic polyimide: This material in the three formulas to be described is XU 218, a trademark product of Ciba-Geigy Corp. It is sold commercially as an undiluted solid, which has a stretchable consistency after imbibing some solvent. It has a density of 1.2 grams per cubic centimeter, and is fully polymerized.

The graphite—This material is Micro 850, a trademark product of Asbury Graphite mills, Inc. It has an average particle diameter of 0.50–0.60 microns. A typical formula in accordance with this invention desirably will have graphite at a level somewhat near the 48% by volume figure which is the state of the art critical pigment volume concentration (CPVC) for graphite. Vulcan XC 72—This is a conductive furnace carbon black, a trademark product of Cabot Corp.

SOTEX N—Trademark product of Morton Chemical Co., division of Morton-Norwich Products, Inc. A polar solvent compatible dispersant.

Tetrahydrofuran (THF)—A solvent for the thermoplastic polyimide; compatible with the other ingredients, thereby serving as a diluent.

##### Preferred Formula

The following materials in the amounts shown were combined with stirring to disperse the graphite for 5 to 10 minutes in a high-speed mixer, cooled with a water jacket. The order is not essential and a full solution is readily achieved. Preferably the thermoplastic polyimide is first solubilized in the tetrahydrofuran. The other ingredients are then added. Once mixed, further mixing appears detrimental.

The resistivity of the final layer 3 from this formula is in the order of magnitude of 1 ohm-cm.

| Component               | Pbw  | Density | Volume |
|-------------------------|------|---------|--------|
| XU 218                  |      |         |        |
| Thermoplastic Polyimide | 4.2  | 1.2     | 3.5    |
| PI 2560                 | 31.2 | —       | —      |
| Thermosetting Polyimide | 11.5 | 1.43    | 8.0    |
| Precursor               |      |         |        |
| N—methyl-2-pyrrolidone  | 14.7 | —       | —      |
| Xylene                  | 5.0  | —       | —      |
| Micro 850 Graphite      | 22.9 | 2.2     | 10.4   |
| Tetrahydrofuran         | 80   | —       | —      |

##### Earlier Formula-1 ohm-cm

This formula preceded the preferred formula and achieved a layer 3 having resistivity of about 1 ohm-cm, a characteristic believed to be near the low end of a range of operability in a thermal ribbon 1 of the general type described. The amounts shown were combined with stirring as described for the preferred formula.

| Component               | Pbw  | Density | Volume |
|-------------------------|------|---------|--------|
| XU 218                  |      |         |        |
| Thermoplastic Polyimide | 2.6  | 1.2     | 2.2    |
| PI 2560                 | 15.9 | —       | —      |
| Thermosetting Polyimide | 5.9  | 1.43    | 4.1    |
| Precursor               |      |         |        |
| N—methyl-2-pyrrolidone  | 7.5  | —       | —      |
| Xylene                  | 2.5  | —       | —      |
| Micro 850 Graphite      | 35.1 | 2.2     | 15.9   |
| Vulcan XC 72            |      |         |        |
| Conductive Carbon Black | 5.4  | 1.8     | 3.0    |
| Tetrahydrofuran         | 90.0 | —       | —      |
| N—methyl-2-pyrrolidone  | 5.0  | —       | —      |

-continued

| Component               | Pbw | Density | Volume |
|-------------------------|-----|---------|--------|
| (Additional to PI 2560) |     |         |        |

## Earlier Formula-10 ohm-cm

This formula preceded the preferred formula and achieved a layer 3 having resistivity of about 10 ohm-cm, a characteristic believed to be near the high end of a range of operability in a thermal ribbon 1 of the general type here described. The amounts shown were combined with stirring as described for the preferred formula.

| Component               | Pbw   | Density | Volume |
|-------------------------|-------|---------|--------|
| XU 218                  |       |         |        |
| Thermoplastic Polyimide | 8.4   | 1.2     | 7.0    |
| PI 2560                 | 4.8   | —       | —      |
| Thermosetting Polyimide | 1.8   | 1.43    | —      |
| Precursor               |       |         |        |
| N-methyl-2-pyrrolidone  | 2.3   | —       | —      |
| Xylene                  | 0.7   | —       | —      |
| SOTEX N                 | 0.3   | 1.00    | 0.3    |
| Micro 850 Graphite      | 20.6  | 2.2     | 9.4    |
| Tetrahydrofuran         | 111.0 | —       | —      |
| N-methyl-2-pyrrolidone  | 5.0   | —       | —      |
| (additional to PI 2560) |       |         |        |

## Stainless Steel

The stainless steel is commercially obtained in bulk amounts at the 0.5 mil (0.001270 cm) thickness. As so obtained, it has a clean, smooth surface.

## Silicon Dioxide

The stainless steel is introduced into a vacuum-deposition chamber. One wide surface of the steel is presented to be coated. Standard procedures are followed. The chamber is evacuated and silicon dioxide is heated until it evaporates to gas and then deposits on to the steel surface present. Deposition is terminated when the thickness is observed at 80 angstroms. The chamber is a standard, commercially available device in which material to be evaporated is heated by an electron beam. A standard, associated crystal monitor device is simultaneously coated and it produces a distinctive signal upon being coated to the designated thickness. This control is not thought to be particularly precise, and 80 anstroms should be understood as an order-of-magnitude dimension.

## Resistive Layer Application

The steel is flattened on a sturdy, highly polished, flat surface, silicon dioxide side up. The preferred formula was applied and doctored to the desired 0.3 mil (0.000762 cm) dry thickness by moving a coating rod having an external wire wound in a helix across the surface. The rod is sturdy stainless steel and the coating thickness is a function of material passed by the spacing between the helical ridges of the wire wrap. (The doctoring device used is a commercially obtained R.D.S. Laboratory Coating Rod, No. 28, which provides a wet thickness of 2.52 mil [0.0064008 cm]). This material solidifies at ordinary room conditions in about one minute, primarily from loss of the highly volatile THF.

The steel as coated is then placed on a controlled heater in the nature of a griddle with the coated side up. It is first heated for 15 minutes at 176° F. (80° C.). Then,

on the same or a second griddle heater, the coated plate is similarly subjected to heating for 15 minutes at 248° F. (120° C.). Then, the heating is similarly applied for 15 minutes at 320° F. (160° C.). At this point, the coating appears free of all dispersants, which have been expelled by the heat. Heat is then applied in the same manner for 1 hour at 335° F. (about 168° C.), which is effective to polymerize the precursor of polyimide to the polyimide.

After cooling the steel has the then finished resistive layer 3 adhering to the silicon dioxide intermediate layer 5.

## Ink Layer Formulations

15 One ink layer formula is applied as a melted liquid and the other is applied as a dispersion in solvent. At room temperature, the ink is a solid. The ink formulation is not an essential contribution of this invention. Nevertheless, Ink Formula 1 below is the inventive contribution of the inventor of this application.

20 Each of the following two formulations have different characteristics as described and are generally equally preferred since adequate embodiments of this invention may employ inks having various characteristics.

25 Both formulas satisfy the following minimum criteria for inks for the thermal ribbon, involved. (1) Solid at room temperature; (2) Strong as solid (optional depending upon use in given reinking system); (3) Homogeneous as solid; (4) Reproducible melting point (in the general range of 70° C. to 100° C.); (5) Rapidly produced low viscosity near melt temperature (in the general range between 1 and 10<sup>3</sup> cps); (6) Homogeneous as a liquid; (7) Fed well and rapidly through applicator (optional depending upon inking or reinking conditions and type of applicator); (8) Uniformly coats metal in thin film (about 0.2 mil or more); (9) Releases from metal or other substrate during printing; (10) Jet black with high optical density; and (11) Smudge resistant as printed characters.

30 The following formula, Ink Formula 1, functions as an interactive combination to achieve the foregoing objectives. In this formula the sucrose acetate isobutyrate appears to make the following contributions: (1) Provides abrupt change in viscosity with temperature; (2) Provides stability during heat exposure; (3) No vaporization during heating; (4) At melt temperature, high solvent action on ethyl cellulose, enhancing compatibility and functionality of the ink; (5) Very high gloss and good adhesion to paper; (6) Suitable to low viscosity inks (7) Compatible with liquid stearic acid; and, (8) Provides lower melting inks than ink of the type of Ink formula 2 below. Also, absence of the sucrose acetate isobutyrate results in poor wetting of the metallic substrate.

35 In this formula the ethyl cellulose appears to make the following contribution: (1) Binder for carbon black thereby improving smudge resistance; and (2) Highly compatible with sucrose acetate isobutyrate and stearic acid. This compatibility in a unique property and directly improves ink deposition and flow from certain applicators. In the absence of ethyl cellulose the ink viscosity would be significantly higher. The ethyl cellulose employed is Hercules Incorporated N-10. The N denotes an ethoxyl content of 47.5-49.0%. The 10 denotes viscosity in centipoises for a 5% concentration when dissolved in 80:20 toluene:ethanol and measured

at  $25 \pm 0.1^\circ \text{C}$ . In this formula the stearic acid appears to make the following contribution: (1) Lowers the viscosity of the ink (stearic acid alone is about 1 cps at melt temperature of the ink); (2) Amenable to low viscosity inks (3) Compatible with sucrose acetate isobutyrate and ethyl cellulose; and, (4) Lowers the melting point of the ink. In the absence of stearic acid, the higher viscosity results in a tacky ink. Other fatty acids or their derivatives, for example glycerol monostearate and fatty acid amides, may be substituted.

5  
10

| Ink Formula 1                           |     |         |        |
|-----------------------------------------|-----|---------|--------|
| Component                               | Pbw | Density | Volume |
| Sucrose Acetate Isobutyrate             | 9.3 | 1.15    | 8.1    |
| Ethyl Cellulose<br>(Hercules Inc. N-10) | 1.2 | 1.14    | 1.1    |
| Carbon Black                            | 1.3 | 1.8     | 0.7    |
| Stearic Acid                            | 6.0 | 0.839   | 7.2    |

This ink formula is particularly well suited to being deposited as a hot melt during bulk manufacturing or at a printer station adapted to use the ribbon 1 repeatedly.

15

| Ink Formula 2                              |             |
|--------------------------------------------|-------------|
|                                            | % By Weight |
| Versamid 871 (Henkel Corp polyimide resin) | 18          |
| Furnace Carbon Black                       | 2           |
| Triphenyl Phosphate                        | 2           |
| Isopropyl Alcohol                          | 78          |

This is a typical formula for inks developed prior to this invention primarily for a single-use thermal ribbon. The formula is applied as a liquid and the isopropyl alcohol driven off by forced hot air drying. (Alternatively, 60 parts by weight Versamid 940 polyamide resin is added to 8.9 parts by weight carbon black and dispersed in isopropyl alcohol. The alcohol is expelled before any coating step and all coating is by hot melt.)

When Ink Formula 2 is used to reink a reusable ribbon 1 at the typing station in accordance with this invention, it will be applied by being melted. Where the reinking apparatus requires the characteristic of ready flow described in connection with Ink Formula 1, that formula would be used.

Typically, even when ribbon 1 is to be reinked at the typing station, a transfer layer 9 is applied during bulk manufacture. When the layer 9 is Ink Formula 1, it is applied as a hot melt, doctored to yield solid thickness of 0.2 mil (about 0.000508 centimeters), and allowed to cool. When the layer 9 is from Ink Formula 2, it is applied as a dispersion, doctored to yield a dry thickness of 0.2 mil (about 0.000508 centimeters), and the alcohol is driven off by forced air heating.

The bulk ribbon is then slit to the width required for the printer with which it is to be used. Typically, where the ribbon 1 is to be used a single time and discarded, it is wound into a spool and may be encased in a cartridge which fits the printer. The preferred embodiment of this invention has the strength and temperature resistance well suited for reinking and is primarily intended for that purposes. It may be joined in an endless band by abutting ends of the steel and welding or the like. It may also be coiled in a spool, although typically not one as large as for a one-use ribbon, and pulled back and forth indefinitely across the printing station while being reinked in the printer at a station spaced from the printing station.

### Use of the Ribbon

A one-use ribbon 1 in accordance with this invention is used conventionally. Current is applied to the resistive layer 3 in the pattern of the character or shape being printed while the ribbon 1 is continually advanced during printing. When the ribbon 1 has been used once, it is replaced.

A reinked ribbon 1 is printed from in the same manner, but it is used indefinitely. As the ribbon 1 passes the printing station, a part of the ribbon 1 passes a reinking station. Reinking would be by a hot melt application of ink followed by doctoring to the original or desired thickness and cooling to a solid. Preferably only a small amount of the ink would be heated while most of the ink would be stored as a solid until melted during use for reinking. The ink formula typically would be the same as originally applied to the ribbon 1. Tests have shown the preferred embodiment ribbon 1 to have excellent abrasion resistance to normal moving contact with a thermal print head.

It will be apparent that the formulation here disclosed can be varied without departing from the spirit and scope of this invention and that, accordingly, patent coverage should not be limited to the specific details disclosed.

What is claimed is:

1. A ribbon for non-impact thermal transfer printing comprising a thermal transfer layer and a resistive substrate which comprises a thorough mixture of a thermosetting polyimide, a thermoplastic polyimide, and an electrically significant amount of conductive, particulate material.

2. The ribbon as in claim 1 which comprises a metal support layer between said transfer layer and said substrate.

3. The ribbon as in claim 1 in which said conductive, particulate material is graphite.

4. A ribbon for non-impact thermal transfer printing comprising a thermal transfer layer and a substrate comprising a mixture of thermosetting and thermoplastic polyimides and a conductive, particulate material, said substrate having a resistance in the range of between 1 ohm-cm and 10 ohm-cm.

5. The ribbon as in claim 4 which comprises a metal support layer between said transfer layer and said substrate.

6. The ribbon as in claim 4 in which said conductive, particulate material is graphite.

7. The method of making a thermal transfer medium comprising applying to one side of a heat-conductive lamination a mixture of a precursor of a thermosetting polyimide, a thermoplastic polyimide, and a particulate filler material dispersed in a dispersant, heating said applied mixture to expell the dispersant of said mixture, heating said applied mixture to polymerize said precursor, coating a thermal ink formula as a liquid on the other side of said lamination, and then solidifying said applied liquid as a thermal ink.

8. The method as in claim 7 in which said dispersant comprises N-methyl-2-pyrrolidone.

9. The method as in claim 8 in which said dispersant also comprises an organic solvent for said thermoplastic polyimide.

10. The method as in claim 7 in which said particulate filler material is graphite.

11. The method as in claim 8 in which said particulate filler material is graphite.

12. The method as in claim 9 in which said particulate filler material is graphite.

\* \* \* \* \*